

Feb. 7, 1961

D. MORGESTERN

2,970,365

NEEDLED FABRIC AND METHOD

Filed Aug. 4, 1958



FIG. 1



FIG. 2



FIG. 3



FIG. 4



FIG. 5



FIG. 6

1

2,970,365

**NEELED FABRIC AND METHOD****David Morgenstern, 1056 5th Ave., New York 28, N.Y.****Filed Aug. 4, 1958, Ser. No. 752,937****9 Claims. (Cl. 28—72.2)**

This invention relates to a new process for manufacturing a fibrous sheet material simulating felt, and more particularly to a novel needled fabric and to the method of making same from normally unfeltable fibers.

A prerequisite for making felt by conventional felting techniques is the employment of feltable fibers. Such fibers, including wool, goat hair and other animal fibers, have a substantial curl and even more important a rough surface which allows the fibers to interlock or interfelt into a felt having substantial strength. Except in admixture with feltable fibers, the vegetable fibers like cotton, the synthetic fibers like rayon, nylon, etc., and even some animal fibers cannot be felted satisfactorily because the characteristically smooth surfaces of these fibers slide upon one another too readily for interfelting.

Non-woven fabrics resembling felt can be made from non-felting fibers by needling. In this method a fiber bat is subjected to many transverse strokes by notched needles which catch fibers during their movement through the thickness of the fleece in one direction, and leave the fibers entangled into a needled fabric. This particular method has the objection that many strokes have to be applied to give some strength to the fabric, and the higher the number of strokes the stiffer the fabric becomes. In order to apply the multitude of strokes needed to give the fabric some strength, the bat or web of heavy fleece has to travel at an extremely low speed, which makes the process very costly.

Needled fabrics suffer from a most serious disadvantage of low strength especially when the fiber bat is not very thick and heavily needled. To avoid this disadvantage many strengthening expedients have been suggested. According to one such method a fibrous fleece is placed over one or both surfaces of a woven fabric and subsequently needled, whereby the woven fabric is integrally embedded and made part of the needled "felt." The woven fabric supplies strength and stability to the needled "felt." This method requires a large number of needle strokes to combine the fibers with the woven fabric which again stiffens the needled fabric, creates lumps and distortion of the needled fabric by pushing out individual threads during the movement or punching thrust of the needles and increases the cost of the product. Still another method involves employment of a potentially adhesive resin in fiber form as part of the fiber mix, needling, and subsequently heating the needled fabric to a temperature whereat the resinous fibers become sufficiently tacky to adhere to the other fibers in the needled fabric.

Needless to say each of the above expedients for forming a strong coherent needled fabric suffers from serious disadvantages.

The principal object of the instant invention is to provide a novel needled fabric of high strength and dimensional stability.

Another object of the instant invention is to provide

2

a process for producing a novel needled fabric of high strength and dimensional stability.

Still a further object of the instant invention is to provide a process for producing a needled fabric of predetermined thickness, strength and dimensional stability.

These and still other objects and advantages will be apparent from the detailed description which follows.

Briefly stated the process of the instant invention contemplates: forming a fleece of fibers, coating the surface with an adhesive binder to form a thin surface layer of bonded fibers, drying said surface and then needling the unbonded fiber fleece through the layer of dried adhesive to form a needled fabric. A single needling operation on each side is sufficient to achieve good "felting" or interlocking of the fibers, and to create a needled fabric of great softness and drape, yet having considerable strength and dimensional stability.

Although the needling makes multitudinous perforations in the adhesively bonded layer of fibers and actually masks this bonded layer from visual discernment thereof, the integrity of the bonds appears in the final needled fabric. As compared to the same fabric made without a surface layer bonded by adhesive, there is substantially increased strength and dimensional stability depending largely upon the amount and character of the adhesive bond. Moreover, the strength and dimensional stability of the ultimate needled fabric can be predetermined within wide limits according to which of the several preferred modes of the instant invention is employed, and 30 the amount of adhesive employed. By and large, at least 30% of the strength and dimensional stability of the needled fabric is derived from the adhesive, and the balance from the needling action.

For a better understanding of the invention, these 35 preferred embodiments will be described in connection with the attached drawing wherein:

Figure 1 is a diagrammatic view of a fiber fleece with one surface sprayed with a liquid binder.

Figure 2 is a vertical view of the sprayed fiber fleece 40 of Figure 1 after needling.

Figure 3 is a vertical view of two fleeces, each sprayed on one side and plied together with the sprayed surfaces placed face to face.

Figure 4 shows the two plied fleeces of Figure 3 after 45 needling.

Figure 5 is a vertical view of two plied fleeces both sprayed on each side.

Figure 6 is a diagrammatic view of the two plied fleeces of Figure 5 during needling.

50 Referring now to Figure 1 of the drawing, there is shown a fiber fleece 7 such as produced by air deposition or by cards or garnettes. One side or surface 6 of the fleece is shown spray coated with a liquid binder and thereafter dried. Figure 2 shows the same coated fleece 55 7 after needling. The needling operation has forced individual fibers 8 through the bonded surface layer 6, causing fibers 8 to protrude to the reverse side of layer 6, and in effect form a new outermost surface layer 9, hiding the existence of adhesive bonded layer 6 from visual discernment.

Numerous variations on the basic invention as illustrated in Figures 1 and 2 are possible. Thus, for example, both surfaces of the initial fleece may be coated with a binder prior to needling. A particularly desirable 65 variation is illustrated in Figures 3 and 4 where two layers of fleece 17, 17', each having an adhesive coated outer layer 6, 6', are placed face to face and then dried to set the adhesive. The drying process can be accomplished in any conventional manner, with or without pressure, depending on whether a lofty or firmer "felt" is to be achieved. Thereafter, needling in one direction forces

fibers 8 from the upper layer 17 into lower layer 17', and a second needling in the opposite direction forces fibers 8 from layer 17' into layer 17 thereby thoroughly interlocking 17, 17' into an integral needled fabric with an adhesively bonded layer embedded at the center of the needled fabric. As shown in Figures 5 and 6, a thinner spray of binder liquid 10 may advantageously be applied to one or both outer surfaces prior or after needling in order to prevent loose, easily removed fibers from being present on the surface of the ultimate needled fabric. In Figure 6, a pair of needles 11, 12 are diagrammatically illustrated.

For best results, the fleece employed for the practice of the instant invention should range in weight between about 0.50 to 7.0 oz. per square yard of single layer. Heavier fabrics than 7 oz. can be built up by employment of multiple layers in the manner illustrated by Figures 3, 4. In contrast, a light but strong needled fabric can be made by needling a single layer of fleece adhesively bonded initially on both surfaces.

The fleece itself can be composed of any fiber: animal, like cattle hair, horse hair, wool, etc.; vegetable, like cotton, linen, piama, cocoa, etc.; mineral, like asbestos, glass, metal, etc.; or synthetic, like rayon, acetate, nylon, etc.; or any desired fiber mixture. Although non-felting fibers are most generally contemplated, wool and other felting fibers can be employed.

The binder liquid is also capable of wide variations. It may be an aqueous or non-aqueous solution emulsion or dispersion of adhesive or of latently adhesive material which upon drying or heating forms an adhesive bond. Thus, for example, known adhesives include: rubber (natural and synthetic), vinyl resins, isocyanate resins, polyamides, polyacrylates, and others.

Suitable solvents for the binder liquid include water or organic volatile solvents such as lower alkanols, hydrocarbons, ketones and the like, or mixtures thereof. Alternatively, no extraneous solvent need be employed when the binder substance is a normally liquid monomer or polymer which forms a solid adhesive in the course of drying or curing. If desired, a curing agent can be incorporated into the binder liquid to speed up setting of the adhesive during the drying or heating. In addition, the binder liquid can incorporate up to 35% by weight of thermosetting resins such as melamine formaldehyde precondensates for imparting other properties as desired. The liquid binder is preferably applied to the fleece by spraying through conventional spray nozzles.

However, the binder liquid should not excessively penetrate the fiber fleece since the object is to form a thin surface layer of bonded fibers. To achieve this objective, the fleece should be sprayed with that amount of binder liquid which will deposit non-volatile binder solids ranging from about 0.05 to 1 times the weight of the fleece.

The drying and setting of the adhesive binder can be accomplished by carrying the sprayed fleece over or between heated rolls with or without the application of pressure, or by carrying the fleece through a drying oven supported otherwise unpressured. After drying is completed, only the thin layer of fibers affected by the binder are chemically bonded into a thin core or stable layer through which free fibers from the remainder of the fleece are forced by subsequent needling. As has been indicated, one needling operation on each side is sufficient to achieve a good "felting" or interlocking of the fibers, and to create a strong, stable "felt" with great softness and drape.

The product, either before or after finishing and needling in accordance with the present invention, can be subjected as desired to other treatments such as printing, dyeing, calendering, etc., or the like. If the liquid binder applied is of a thermoplastic nature, the needled fabric can be subjected to heat, making the adhesive tacky. This subsequent treatment will add firmness to

the needled fabric by bonding the transversely extending fibers 8 to layer 6 at the needle perforations of layer 6 where fibers 8 contact the adhesive bonding the original surface layer 6.

5 The novel process of the present invention is considerably less expensive than felting. A variety of fibers can be used which have no felting properties, yet the results achieved will be very similar to those of genuine felt, especially as far as dimensional stability and strength are concerned. The density of the product made by practice of this invention can be controlled to a greater degree than in conventional felting or needling processes. The same applies to the softness and hand of the fabric as well as air permeability, all of which can be controlled 10 to any desired degree.

15 Products made in accordance with the practice of the instant invention have an almost unlimited amount of uses in the garment and industrial fields. The products are not intended to merely substitute for existing fabrics. Practice of the instant invention will result in much superior products more suitable for certain end uses than textiles now in existence.

20 The following specific examples further illustrate the practice of the instant invention.

#### Example I

To a single ply of 4 oz. per sq. yd. cotton fiber fleece apply on one side 2 oz. per sq. yd. liquid binder the pre-plasticized polyvinyl chloride emulsion (40% solids content) shown below:

|                                              | Wet wt. |
|----------------------------------------------|---------|
| Polyvinyl chloride emulsion 55% total solids | 100     |
| Butyl benzyl phthalate                       | 20      |
| Water                                        | 62.5    |
|                                              | 182.5   |

Dry the coating at 250° F. for five minutes. After drying, pass the coated fiber fleece through the needling machine with the uncoated side of the fleece towards the needles.

#### Example II

To a 3 oz. per sq. yd. nylon fiber fleece apply a 1 oz. per sq. yd. spray coat of a blend of acrylic resin emulsion and casein solution (40% solids) as shown below:

|                                          | Wet wt. |
|------------------------------------------|---------|
| Acrylic resin emulsion 46% total solids  | 100     |
| (Rhoplex B-15)                           | 100     |
| Ammonia casein solution 20% total solids | 20      |
|                                          | 120     |

Dry the coated fleece two minutes at 250° F. Repeat the 1 oz. per sq. yd. spray coating on the uncoated side 55 of the fiber fleece and dry as before. After the second coat has been dried, pass the coated fleece through the needling machine twice, turning the piece over between passes.

#### Example III

60 Apply a 1 oz. per sq. yd. spray coat to one side each of two 2 oz. per sq. yd. acetate-nylon blended fiber fleeces, each fleece consisting of 50% acetate staple fiber and 50% nylon staple fiber. The spray coating formula is shown below:

|                                             | Wet wt. |
|---------------------------------------------|---------|
| Polyvinyl acetate emulsion 55% total solids | 100     |
| Tributyl phosphate                          | 35      |
| Water                                       | 90      |
|                                             | 225     |

70 40% total solids.

75 While the sprayed fleeces are wet, they are plied together with the adhesive faces against each other. The plied fleeces are then dried at 250° F. for two minutes,

after which the plied stock is passed through heated rolls using the following conditions:

Temperature \_\_\_\_\_ ° F. 350  
 Gap between rolls \_\_\_\_\_ inch. 0.020  
 Roll surface speed \_\_\_\_\_ ft. per minute. 15

From the rolls, the plied and pressed fleece is passed through the needling machine twice with the piece being turned over between passes.

*Example IV*

To two 2.5 oz. per sq. yd. wool and nylon blended fleeces apply a 1.5 oz. per sq. yd. spray coat of the compounded nitrile rubber, formulation shown below:

|                                                            | Wet wt. |
|------------------------------------------------------------|---------|
| Nitrile rubber latex 40% total solids [Hevea (Int. Latex)] | 200     |
| Zinc oxide                                                 | 4       |
| Sulfur                                                     | 2       |
| Zinc dibutyl dithiocarbamate                               | 2       |
| Alkyl aryl polyether alcohol (Triton X-100)                | 2       |
| Water                                                      | 15      |
| 225                                                        |         |

40% total solids.

After spraying, the fleeces are placed against each other so that the binder coated surfaces meet. The plied material is then dried at 250° F. for three minutes. After drying, the plied and bonded fiber fleeces are passed through the needling machine twice. The piece is turned over between passes. The needled piece is now cured at 275° F. for one hour.

*Example V*

To two 3 oz. per sq. yd. wool fiber fleece apply 1.0 oz. per sq. yd. of polyamide binder of the formula shown below:

|                                                   | Wet wt. |
|---------------------------------------------------|---------|
| Polyamide resin solution 10% total solids (Zytel) | 200     |
| Citric acid                                       | 1       |
| 201                                               |         |

10% total solids.

Place the coated fiber fleeces together in such a manner that the binder coated faces are against each other. The plied and bonded fiber fleece is then oven dried at 250° F. for three minutes. After drying, a top coat of 0.5 oz. per sq. yd. of polyamide binder of the same formulation used in the first spray operation is put on one side of the bonded fiber fleece. After drying, for one minute at 250° F., the same operation is repeated on the opposite side of the fiber fleece. After drying, the bonded fiber fleece is passed through the needling machine twice. The piece is turned over between passes. When this operation has been completed, the bonded and plied fiber fleece is oven cured for 10 minutes at 300° F.

*Example VI*

To two 2 oz. per sq. yd. fiber fleeces of 60% nylon staple fiber and 40% cotton staple fiber, apply a 1 oz. per sq. yd. spray coat of nitrile rubber latex blended with melamine-formaldehyde resin solution as shown in formula below:

|                                                            | Wet wt. |
|------------------------------------------------------------|---------|
| Nitrile rubber latex 40% total solids [Hevea (Int. Latex)] | 200     |
| Zinc oxide                                                 | 4       |
| Sulfur                                                     | 2       |
| Alkyl aryl polyether alcohol (Triton X-100)                | 2       |
| Melamine formaldehyde resin 80% total solids               | 25      |
| Water                                                      | 50      |
| 283                                                        |         |

40% total solids.

After spraying, the coated fiber fleeces are oven dried for two minutes at 250° F. Next the two coated fiber fleeces are plied together with the coated sides against each other. This operation is performed by passing the fleeces through the needling machine twice. The piece is turned over between passes. After needling, the plied piece is cured in an oven at 275° F. for one hour.

*Example VII*

10 To two 2.5 oz. per sq. yd. nylon fiber fleeces apply a 1.5 oz. per sq. yd. spray coat of polyurethane binder using the formula shown below:

|                                   | Wet wt. |
|-----------------------------------|---------|
| Toluene diisocyanate              | 180     |
| Polyester resin [PFR-4 (Barrett)] | 1000    |
| Ethyl acetate                     | 590     |
| Toluol                            | 590     |
| Methyl diethanolamine             | 20      |
| 2380                              |         |

50% total solids.

The coated fiber fleece is now plied together with the coated surfaces against each other. The plied fiber fleece is oven dried at 200° F. for five minutes. After drying, a top coat of 0.5 oz. per sq. yd. of plasticized soya protein binder is sprayed on only one side of the fiber fleece. The formula for this top coating is shown below:

|                     | Wet wt. |
|---------------------|---------|
| Soya protein        | 100     |
| Ammonia 26° Bé.     | 20      |
| Water               | 480     |
| Polyethylene glycol | 25      |
| 625                 |         |

20% total solids.

After spraying, the plied and coated fiber fleece is dried for one minute at 250° F. The top coating spray and drying is repeated on the opposite side of the piece. After top coating both sides, the piece is pressed through rolls under the conditions shown below:

|                    |                |       |
|--------------------|----------------|-------|
| Roll temperature   | ° F.           | 350   |
| Gap between rolls  | inch.          | 0.006 |
| Roll surface speed | ft. per minute | 20    |

When the piece has been rolled, it is passed through the needling machine twice. The piece is turned over between passes through the machine. After needling, the bonded fiber fleece is cured at 250° F. for 20 minutes in an oven.

What is claimed is:

1. A needled fabric comprising a web of a plurality of fleece consisting wholly of loose fibrous material having adhesive distributed within said loose fibrous material in the form of a layer coextensive with and parallel to the planar surfaces of the web, some of the fibers of said web of fibrous material being randomly arranged and some of the fibers of said fibrous material extending through said adhesive layer and through said web, the latter fibers extending substantially normal to the planar surfaces of said web, said fabric being an integral structure.

2. A needled fabric comprising a web of a plurality of fleeces consisting wholly of loose fibrous material, at least one of said fleeces having adhesive distributed within said loose fibrous material in the form of a layer coextensive with and parallel to the planar surfaces of the web, some of the fibers of said web of fibrous material being randomly arranged and some of the fibers of said fibrous material extending through said adhesive layer and through said web, the latter fibers extending substantially normal to the planar surfaces of said web and are adhesively bonded to said adhesive layer, said fabric being an integral structure.

3. A needled fabric weighing from 0.30 to 7.0 oz. per

square yard comprising a web of a plurality of fleeces consisting wholly of loose fibrous material having adhesive distributed within said fibrous material in the form of a layer coextensive with and parallel to the planar surfaces of the web and in an amount of from 0.05 to 1.00 times the weight of said fibrous material, some of the fibers of said fibrous material being randomly arranged and some of the fibers of said fibrous material extending through said adhesive layer and through said web, the latter fibers extending substantially normal to the planar surfaces of said web, said fabric being an integral structure.

4. A needled backing-free fabric comprising a web consisting wholly of loose fibrous material having adhesive distributed in the form of a layer coextensive with and parallel to the planar surfaces of the web, some of the fibers of said fibrous material being randomly arranged and some of the fibers of said fibrous material extending through said adhesive layer and through said web, the latter fibers extending substantially normal to the planar surfaces of said web, said fabric being an integral structure.

5. Method of producing a needled fabric of integral structure which comprises applying to a substantially flat fleece consisting wholly of loose fibrous material a coating of liquid adhesive material thereby bonding some of the surface fibers of the fibrous material to each other to form a thin surface layer of adhesively bonded fibers coextensive with and parallel to the planar surfaces of the fleece, drying the coating of adhesive material, and then needling said fleece to form a web wherein some of the fibers of said fibrous material are randomly arranged and some of the fibers extend substantially normal to the planar surfaces of said web and through the dry adhesive layer.

6. Method of producing a needled fabric of integral structure which comprises applying to a substantially flat fleece free of fabric backing and consisting wholly of loose fibrous material a coating of liquid adhesive material thereby bonding some of the surface fibers of the fibrous material to each other to form a thin surface layer of adhesively bonded fibers coextensive with and parallel to the planar surfaces of the fleece, drying the coating of adhesive material and then needling said fleece to form a web wherein some of the fibers of said fibrous material are randomly arranged and some of the fibers extend substantially normal to the planar surfaces of said web and through the dry adhesive layer.

7. Method of producing a needled fabric of integral structure which comprises applying to a substantially flat fleece free of fabric backing and consisting wholly of loose fibrous material a coating of liquid adhesive material in an amount of from 0.05 to 1.0 times the weight

of said fibrous material thereby bonding some of the surface fibers of the fibrous material to each other to form a thin surface layer of adhesively bonded fibers coextensive with and parallel to the planar surfaces of the fleece, drying the coating of adhesive material, and then needling said fleece to form a web wherein some of the fibers of said fibrous material are randomly arranged and some of the fibers extend substantially normal to the planar surfaces of said web and through the dry adhesive layer.

10 8. Method of producing a needled fabric which comprises applying a coating of liquid thermoplastic adhesive to a surface of at least one of a plurality of substantially flat fleeces consisting wholly of loose fibrous material so that some of the surface fibers of the fibrous material of the fleece are bonded to each other to form a thin surface layer of adhesively bonded fibers, assembling the fleeces with the adhesive-carrying surface of the coated fleece in contact with another fleece, drying 15 the adhesive, and then needling the laminate whereby some of the fibers of the fleece are randomly arranged and some of the fibers extend substantially normal to the planar surfaces of the laminate and through the dry adhesive layer to the surfaces of said fleeces, and then heating 20 the needled laminate whereby the normally extending fibers are bonded to the adhesive layer.

25 9. Method of producing a needled fabric which comprises applying a coating of liquid adhesive to a surface of at least one of a plurality of substantially flat fleeces 30 consisting wholly of loose fibrous material so that some of the surface fibers of the fibrous material of the fleece are bonded to each other to form a thin surface layer of adhesively bonded fibers, assembling the fleeces with the adhesive-carrying surface of the coated fleece in contact with another fleece, drying the adhesive, and then needling the laminate whereby some of the fibers of the 35 fleece are randomly arranged and some of the fibers extend substantially normal to the planar surfaces of the laminate and through the dry adhesive layer and then heating the needled laminate whereby the normally extending fibers are bonded to the adhesive layer.

#### References Cited in the file of this patent

##### UNITED STATES PATENTS

|           |                  |               |
|-----------|------------------|---------------|
| 1,345,693 | Pye              | July 6, 1920  |
| 2,249,888 | Dodge            | July 22, 1941 |
| 2,794,238 | Dildilian et al. | June 4, 1957  |
| 2,794,759 | Dildilian        | June 4, 1957  |
| 2,845,687 | Howard           | Aug. 5, 1958  |

##### FOREIGN PATENTS

|         |               |                |
|---------|---------------|----------------|
| 556,186 | Great Britain | Sept. 23, 1943 |
| 748,136 | France        | Apr. 10, 1933  |